

May 30, 1933.

F. O. W. LOOMIS ET AL

1,911,761

METHOD OF PREPARING BITUMINOUS ROAD SURFACING MATERIALS

Filed June 3, 1931



FIG. 1



FIG. 3



FIG. 2

INVENTORS  
FREDERICK O. W. LOOMIS  
DANIEL M. LOOMIS  
BY *J. D. Loomis*  
ATTORNEY

Patented May 30, 1933

1,911,761

# UNITED STATES PATENT OFFICE

FREDERICK OSCAR WARREN LOOMIS AND DANIEL MACKAY LOOMIS, OF MONTREAL,  
QUEBEC, CANADA

## METHOD OF PREPARING BITUMINOUS ROAD SURFACING MATERIALS

Application filed June 3, 1931, Serial No. 541,837, and in Canada April 24, 1931.

This invention relates to the preparation of road surfacing materials and particularly to the coating and mixing of the mineral particles of the aggregate. In preparing road surfacing materials in accordance with prevailing methods wherein the bitumen is used in the form of a watery emulsion, the crushed stone or similar aggregate is initially placed in a mixer and agitated to effect the desired distribution of the particles of varying sizes. The bituminous emulsion is then added and the mixing operation continued to distribute the bitumen. The mixing is usually carried out in a pug mill or similar mixer equipped with revolving blades or in a revolving drum which may or may not be equipped with mixing blades. Generally speaking, these and similar methods of mixing now in use are not suitably adapted to the use of bituminous emulsions and do not produce satisfactory results. When a pug mill or bladed mixer is used the pugging or blading action causes an immediate breaking down of the emulsion which interferes with proper distribution of the bitumen and produces a dry appearing mix of unsatisfactory characteristics. In some instances the fine particles of the aggregate may absorb and break down the emulsion by capillary action and this also produces a defective, dry appearing mix containing balls of bitumen. In other instances where the aggregate used is of a composite nature, including, for example, coarse particles of crushed stone and fine particles of sand, there is a differential selection by the bitumen which generally leaves the sand uncoated. In an effort to avoid these difficulties it has been a practice to leave out the fines and to carry out the mixing operation in a rotary drum without the use of mixing blades. This produces a defective mix in that the coating of bitumen covering the mineral particles lacks stability and adhesiveness.

The improved method provided in accordance with this invention overcomes these difficulties and enable bituminous emulsions to be successfully used in the production of a satisfactory mix in which the bitumen is uni-

formly distributed over the surfaces of the coated particles and possesses the desired qualifications with respect to stability and adhesiveness.

In accordance with the preferred method of carrying out the invention the aggregate is initially separated into coarse and fine particles, the basis on which the separation is carried out being dependent upon the nature of the aggregate and the type of mix to be produced. After the separation the coarse particles are fed at a uniform rate into a revolving drum preferably equipped with suitable blades arranged so that the coarse particles are given a rolling and rotating motion while travelling lengthwise through the drum. During their progress through the drum the coarse particles are passed beneath one or more sprays of bituminous emulsion and are uniformly coated since the rolling and rotating motion of the particles causes the various surfaces thereof to be exposed to the sprays. The finer particles resulting from the initial separation are then sprayed onto the coated particles and the finished mix is then discharged after being subjected to a few revolutions of the drum.

A simple form of apparatus capable of being used in carrying out this invention is shown diagrammatically in the accompanying drawing wherein

Figure 1 is a view of the apparatus in side elevation, a part of the mixing drum being broken away to disclose the means provided for spraying the bituminous emulsion and the finer particles of the aggregate onto the coarser particles.

Figure 2 is a transverse sectional view through the mixing drum illustrating diagrammatically the manner in which the bituminous emulsion is sprayed onto the coarse particles of the aggregate. In this view the means provided for spraying the finer particles of the aggregate are omitted.

Figure 3 is a cross sectional view through the drum illustrating the manner in which the finer particles of the aggregate are sprayed onto the coated coarse particles.

The initial separation of the aggregate may be regulated to give any desired ratio

of coarse to fine particles. Generally speaking, the separation should yield 70% to 90% of the aggregate as coarse particles and the remainder as "fines". In one instance the aggregate used consisted of all sizes of particles of crushed limestone ranging from those passing through a 200 mesh screen up to those just capable of passing through a circular opening having a diameter of 1½ in. This aggregate was separated into coarse particles of a size exceeding ¼ in. and fine particles of a size less than ¼ in. This basis of separation usually affords 75% to 80% coarse particles and 25% to 15% "fines".

When using an apparatus such as shown in the present drawing the coarse particles resulting from the initial separation are placed in a storage bin 5 equipped with a discharge controlling gate 6 while the fine particles are placed in a similar discharge bin 7 equipped with a controlling gate 8.

The coarse particles are delivered from the bin 5 to the hopper 10 of a mechanical feeder which is herein shown as including an endless conveyor 11 driven by a belt connection 12 from a main drive shaft 13. The conveyor 11 functions to deliver the coarse particles, at a uniform rate, to the feed hopper 14 of a revolving drum 15 which is preferably equipped with mixing blades 16. As herein shown the drum is provided with annular track members 17 mounted on supporting rollers 18 so that the drum has a slight downward inclination towards the discharge opening which is located at the end remote from the feed hopper 14. The drum supporting rollers 18 are carried by suitable shafts 19 and one or both of these shafts may be driven from a motor 20 through any suitable form of gearing such as that indicated at 21. During rotation of the drum the coarse particles progress towards the discharge end by a spiral motion in the course of which the various surfaces of the particles are exposed to the action of the spraying devices 22 which are supplied with bituminous emulsion through a supply pipe 23 connected to the discharge side of a suitable pump 24 which is also driven by a belt 25 from the main drive shaft 13. The pump is equipped with an intake pipe 24a and a funnel 24b. The bitumen is delivered to the funnel through a supply pipe 24c equipped with a valve 24d and leading from an overhead supply tank 24e. This arrangement enables the operator to make sure that an adequate flow of emulsion is maintained during operation of the apparatus. The rate at which the emulsion is fed to the spray pipes is determined by the speed of the pump and the opening of the valve 24d is regulated to keep the funnel about half full.

The fine particles of the aggregate pass

from the bin 7 into a feed hopper 26 and from thence onto the receiving end of a belt conveyor 27 having its discharge end located within the drum 15. The conveyor 27 delivers the fine particles through a chute 28 into the path of a blast of air coming from an air nozzle 29 connected to the discharge side of a blower 30 which is driven by a belt connection 31 from the main drive shaft 13. From the disclosures of Figures 1 and 3 it will be noted that the fine particles are sprayed onto the coarse particles after the latter have been passed beneath the spray devices 22 and coated with the bituminous emulsion. After the spraying of the finer particles the resulting mix is subjected to a few revolutions of the drum before passing outwardly through the discharge opening at the lower end of the drum. The conveyor 27 is driven from the shaft 13 through the belt connection 33 and the geared shafts 34 and 35.

When a mixing drum 30 ins. in diameter and 10 ft. long with a fall of 2 ins. in length is revolved at a speed of approximately 18 revolutions per minute the coarse particles will traverse the length of the drum in about 1½ mins. Such a drum will handle from 8 to 12 tons of coarse particles per hour. When using a drum of this character the bituminous emulsion is usually pumped or otherwise supplied to the spray nozzles 22 at a uniform rate of about 80 to 120 gallons per hour. The emulsion may be sprayed through the nozzles by the use of air or steam such as employed in connection with paint sprays or may be simply forced through the nozzle openings by pressure as in the case of water spray nozzles. Generally speaking, it is advisable to provide a number of relatively small sprays 22 in preference to a single large spray since this enables the sprays to be distributed over a greater area and insures that each coarse particle is completely coated during its passage through the drum. The finer particles of the aggregate are preferably delivered into the mixing drum at a uniform rate of from one to three tons per hour by means of the conveyor 27 and the air blast nozzle 29.

When it is desired to apply a heavy coat of bitumen to the coarse particles and to increase the percentage of the fine particles this is accomplished by providing consecutive banks of the emulsion and fine particle sprays. Various expedients such as dampening the coarse or fine particles with water before feeding the same into the drum may be resorted to in order to eliminate differential selection by the bituminous emulsion and to ensure uniform coating of all particles.

The method of operation described in the foregoing may be readily altered or controlled to adapt the same to the use of

different aggregates and bituminous emulsions and to produce various types of finished mixes. For example, bituminous emulsions which are very sensitive to vibrations may be used by reducing the speed of the drum whereas the breaking down of more stable emulsions after contact with the coarse particles may be readily accomplished by accelerating the speed of the drum. Uniform distribution of the bitumen and fine particles in the mix may be obtained by regulating the sprays.

By completely eliminating the fine particles of the aggregate and treating the coarse particles with kerosene or oil, either separately or combined or accompanied by fine material such as hydrated lime, stone dust, etc., before spraying the coarser particles with the bituminous emulsion, a fairly satisfactory material is also produced in accordance with this invention. This material may be improved by steaming the same after the application of the bituminous emulsion. Kerosene, oils or other substances may also be added to the bituminous emulsion before the latter is sprayed onto the coarser particles in order to ensure satisfactory results when the coarse particles are porous or dirty. When the aggregate consists of glassy and dust free stone satisfactory results have been obtained by merely directing streams of bitumen onto the particles instead of employing the sprays previously described since, in this case, the fine spraying of the bitumen is not always necessary.

From the foregoing it will be apparent that the method described herein comprises the following essential steps: (1) separating the aggregate into coarse and fine particles; (2) uniformly coating the coarse particles with bitumen preferably applied in the form of a spray; and (3) spraying the coated coarse particles with the fine particles to retain the bitumen coating of the coarse particles in place thereon. In this process the dividing point between the coarse and fine particles of the aggregate is predetermined so that none of the coarse particles are fine enough to cause the bitumen to congeal, set or break when sprayed thereon. At the same time these coarse particles are small enough to prevent undue "running off" of the bitumen from the surfaces to which it is applied. The distribution and atomization of the sprays is regulated so that the coarse particles are provided with a uniform bitumen coating of the required thickness. Atomization of the bitumen may be effected by placing the bitumen under the required pressure or by the use of compressed air, steam or any other means capable of close regulation. By suitably regulating the spraying of the fine particles of the aggregate it is possible to congeal,

"set", or break the bitumen or bituminous emulsion just sufficiently to preserve the uniformity of the finished mix without destroying the plasticity necessary to easy transportation and laying of the mix.

Having thus described our invention, what we claim is:

1. A method of preparing bituminous road surfacing materials which comprises applying a coating of bituminous emulsion to coarse aggregate particles of such size as to prevent "breaking" or excessive "running off" of the emulsion when applied to said particles and then applying "fines" to the bituminous coatings of the coarse particles with sufficient impact to cause the bitumen of the emulsion to separate out and adhere to the coarse particles.

2. A method of preparing bituminous road surfacing materials which comprises (1) coating coarse particles of an aggregate with a bituminous emulsion applied in the form of a spray while subjecting the particles to gentle agitation sufficient to cause all surfaces of the particles to be exposed to the coating action of the spray, the size of said particles being predetermined to prevent "breaking" or excessive "running off" of the emulsion as it is applied to said particles and (2) then subjecting the coated coarse particles to a spray of finer particles directed thereon with sufficient force to break down the emulsion by impact so that the bitumen of the emulsion is caused to separate out and adhere to the coarse particles to provide the latter with a uniform bitumen coating stabilized by incorporation of the fine particles therein.

3. A method of preparing bituminous road surfacing materials which comprises (1) separating from an aggregate the finer particles which would tend to break down a bituminous emulsion applied to said aggregate (2) coating the remaining coarse particles of the aggregate with a bituminous emulsion and (3) applying the finer aggregate particles of the initial separation to the coated coarse particles with sufficient impact to cause the bitumen of the emulsion to separate out and adhere to the coarse particles.

4. A method of preparing bituminous road surfacing materials which comprises (1) removing from an aggregate the finer particles which would tend to break down a bituminous emulsion applied to said aggregate (2) coating the remaining coarse particles of the aggregate with a bituminous emulsion applied in the form of a spray while subjecting said particles to gentle agitation sufficient to cause all surfaces of the particles to be exposed to the coating action of the spray and (3) then spraying the finer aggregate particles of the initial separation

70

75

80

85

90

95

100

105

110

115

120

125

130

